

# UNITED STATES PATENT OFFICE.

EDUARD LIEBERT, OF BERLIN, GERMANY.

## MANUFACTURE OF EXPLOSIVES.

SPECIFICATION forming part of Letters Patent No. 413,070, dated October 15, 1889.

Application filed July 10, 1889. Serial No. 317,078. (No specimens.)

*To all whom it may concern:*

Be it known that I, EDUARD LIEBERT, a subject of the King of Prussia, German Empire, and a resident of Berlin, Kingdom of Prussia, 5 German Empire, have invented certain new and useful Improvements in the Manufacture of Explosive Compounds, of which the following is a specification.

This invention relates to the manufacture 10 of explosive compounds.

A great disadvantage of nitro-glycerine and the dynamite produced from the same consists in their sensitiveness to blows or shocks and in the property which they possess of 15 congealing or solidifying. In order to obviate these defects, various substances have heretofore been added to the glycerine—such as, for example, nitro-benzoole. Although nitro-benzoole possesses the property of rendering nitro-glycerine less sensitive to blows or 20 shocks and of lowering the freezing-point thereof, it has, on the other hand, the disadvantage of considerably decreasing the explosive force of the nitro-glycerine, and that the 25 mixture leaves behind undecomposed vapors of nitro-benzoole after the explosion, which vapors are much more dangerous when inhaled than the gases produced by the explosion of the nitro-glycerine itself.

30 Isoamyl nitrate has been found to be a substance which, added to nitro-glycerine, presents all the advantages of nitro-benzoole without having the above-mentioned defects.

Nitro-glycerine mixed with five per cent. of isoamyl nitrate does not commence to freeze 35 at thirty-five degrees below zero, its sensitiveness to blows or shocks is much less than that of pure nitro-glycerine, the explosive force is greater than that of pure nitro-glycerine, and, as isoamyl nitrate under certain 40 circumstances is an explosive substance, it will be completely decomposed by the explosion, and the gases produced scarcely differ from those which are produced by the explosion of pure nitro-glycerine, and are not poisonous, 45 as are vapors of nitro-benzoole. Moreover, isoamyl nitrate is cheaper than nitro-benzoole.

A suitable addition to the nitro-glycerine consists of three percent. of isoamyl nitrate, or more. In lieu of adding isoamyl nitrate to 50 the prepared nitro-glycerine, an emulsion of glycerine and isoamyl nitrate or isoamyl alcohol can be nitrated.

What I claim is—

The process of producing a new explosive 55 compound, consisting in adding isoamyl nitrate to the nitro-glycerine, or nitrating a mixture containing glycerine with isoamyl nitrate or isoamyl alcohol.

In witness whereof I have hereunto set my 60 hand in presence of two witnesses.

EDUARD LIEBERT.

Witnesses:

B. ROI,  
A. SIEBER.